

Dec. 4, 1934.

E. B. McCONNELL

1,982,920

PROCESS FOR MAKING ASPHALT

Filed July 3, 1931



Fig. 1



Fig. 2

INVENTOR.  
Elliott B. McConnell  
BY  
Fay, Oberlin & Fay  
ATTORNEYS.

## UNITED STATES PATENT OFFICE

1,982,920

## PROCESS FOR MAKING ASPHALT

Elliott B. McConnell, Cleveland Heights, Ohio,  
assignor to The Standard Oil Company, Cleve-  
land, Ohio, a corporation of Ohio

Application July 3, 1931, Serial No. 548,601

4 Claims. (Cl. 196--74)

A fundamental difficulty in the manufacture of asphalt has centered about the limitation of oxidizing action. In the customary procedure in which petroleum has been distilled, with removal of progressively heavier cuts down to lubricating fractions, and the bottoms or residuum has then been subjected to the action of air as bubbled through a perforated pipe along the bottom of the still, the amount of exposure and contact 10 action has been so limited as to necessitate very prolonged treatment, two or three days for a batch; and besides the draw-back of such a large time factor there is the further difficulty that such prolonged subjection of hydrocarbons to the high 15 temperatures necessary, effects detrimental decompositions tending to erratic and deficient results. In accordance with the present invention, however, it now becomes possible to subject asphalt-forming residuum to a thorough-going oxidation treatment with relatively small time requirement, and besides a continuous type procedure, as opposed to batch-wise, is available.

To the accomplishment of the foregoing and related ends, the invention, then, comprises the 25 features hereinafter fully described, and particularly pointed out in the claims, the following description and the annexed drawing setting forth in detail certain illustrative embodiments of the invention, these being indicative however, of but 30 a few of the various ways in which the principle of the invention may be employed.

In said annexed drawing:

Fig. 1 is a semi-diagrammatic sectional elevation showing apparatus contemplated; and Fig. 2 35 is a similar view of a modification.

A petroleum residuum, as obtained for instance by distilling petroleum and removing the naphtha and progressively heavier cuts on through the lubrication fractions, for example the residuum or bottoms from the distillation of Mid-Continent petroleum as reduced to about 7-8 per cent is, in molten or adequate<sup>v</sup> fluidified form, projected in 40 finely divided spray or atomized condition counter-currently to a supply of air. For such fine division, finely perforated or porous plates or air-atomizer heads may be employed, especially mechanical atomizer heads in which the subdivision of liquid is effected by the pressure applied and the emergence through passages affording a fine 45 breaking up of the liquid body with formation of very small droplets or mist particles as projected into the air. In the form of equipment illustrated in Fig. 1, atomizer-spray heads 2, preferably of fluid-pressure-whirling type are arranged 50 at the top of a suitable chamber or tower 3, and

are supplied by pipe 4 from a source of residuum, for instance a pump 5 serving to provide a requisite distribution pressure. At the bottom of the chamber 3 an air inlet is provided and this may conveniently take the form of a perforated pipe 6 60 connected with a blower or compressor 7, for supply of a body of air in the chamber. At the top an off-take pipe 8 may lead through a condenser 9 to a receiver 10, and if desired an eduction air pump or blower at the end of the vent pipe 11. 65

As above indicated, the residuum, for instance as coming from the final distillation zone, through pipe 12, and at a temperature of around 700° F., or lower, to about 400° F., is fed by the pump 5 to the atomizer heads 2, where it is projected in finely divided atomized form, preferably in whirls, against a rising current of air introduced by pipe 6. As the finely divided residuum or mist-like particles leave the atomizer heads, they are at once enveloped in an abundance of air, and with 70 the elevated temperatures provided and the exaggerated surface exposure, oxidation proceeds effectively. The product collecting at the bottom of the tower may be drawn off through the pipe 13 to tanks, shipping drums, or whatever disposal 75 is desired. In some cases, further treatment may be preferred by recycling the material through the pipe 14, the valves 15 and 16 being closed and the valves 17 and 18 being open. The pump 5 then recycles the material until a sample taken 80 off at the sampling outlet 19, shows the desired specification characteristics. The effluent air proceeds through off-take pipe 8 and the condenser 9 to the discharge pipe 11, any condensable substances being collected in the receiver 10. 85 Temperature control may be maintained as desired by the temperature of the incoming residuum and the air. The air may be cooled in some cases as required, or it may be specially heated, or it may carry the heat acquired in the 90 compressor.

In the form shown in Fig. 2 of the drawing, there is provided in the upper portion of the tower 3' a finely perforated diaphragm 2'. On account of the difficulty in attaining a desirably 100 fine perforation by direct mechanical punching, it is preferable to provide such perforated diaphragm in the form of a porous plate or plates making up a header of sufficient extent, and such plates may be of any suitably porous material, 105 as for example aluminum oxide, porcelain or other ceramic material in which pores may be conveniently formed by proportioning the granular raw material from which the plates are initial- 110

ly molded. Various degrees of size of pore openings may be had in materials of this order. Desirably, a heating means, as for instance a steam coil 20, is provided adjacent the diaphragm 2', 5 for facilitating melting out of residuum which may become solidified or frozen on occasion of temporary shut-down. The tower otherwise may be equipped with a feed supply line 4', with its pump 5' and connection 12' to a source of supply, 10 by-pass 14'. An air supply, in the form of a pump or blower 7' with discharge 6' in the lower portion of the tower is also provided, and an off-take or vent pipe 8', which is desired may lead through a condenser 9' to a receiver 10' and final 15 vent 11'.

Where it is desired to especially heat the air from the compressor, the heater 21 may be applied to the air pipe prior to its entrance into the tower, the heat being applied by any suitable 20 means, such as a furnace or a flue-gas connection.

Other modes of applying the principle of the invention may be employed, change being made as regards the details described, provided the features stated in any of the following claims, or 25 the equivalent of such, be employed.

I therefore particularly point out and distinctly claim as my invention:—

1. A process of making oxidized asphalt, which comprises atomizing petroleum residuum in whirling, non-stratifying form in counter-current flow to air. 80

2. A process of making oxidized asphalt, which comprises atomizing petroleum residuum in whirling, non-stratifying form in counter-current flow to heated air. 85

3. A process of making oxidized asphalt, which comprises circulating petroleum residuum in finely-divided form counter-currently to an air stream while continuously varying the positions of the points of uninterrupted entry of the finely-divided residuum relative to the air stream and withdrawing the oxidized products. 90

4. A process of making oxidized asphalt, which comprises circulating petroleum residuum in finely-divided form counter-currently to a hot air stream while continuously varying the positions of the points of uninterrupted entry of the finely-divided residuum relative to the air stream and withdrawing the oxidized products. 95

ELLIOTT B. McCONNELL. 100